

## UNITED STATES PATENT OFFICE

2,127,001

## TREATMENT OF HYDROCARBONS

Jacque C. Morrell, Chicago, Ill., assignor to Universal Oil Products Company, Chicago, Ill., a corporation of Delaware

No Drawing. Application February 27, 1936,  
Serial No. 66,065

3 Claims. (Cl. 196—10)

This invention relates more particularly to treatment of normally gaseous olefin hydrocarbons to produce liquid polymers therefrom which are particularly suitable for use in the manufacture of high grade high antiknock motor fuel.

More specifically the invention is concerned with a catalytic process whereby certain more chemically reactive constituents of hydrocarbon gas mixtures, such as those produced incidental to the cracking of heavy petroleum oils for gasoline manufacture, are caused to polymerize more or less selectively to produce liquid fractions of limited boiling range and unusually valuable characteristics from a motor fuel standpoint.

Within the past few years the petroleum industry has been continually confronted with the problem of increasing both the quantity and the quality of its motor fuel products, particularly from an antiknock standpoint, and has met the problem largely by cracking the heavier distillate and residual fractions of petroleum produced in the primary distilling processes to produce additional yields of light oil. Fortunately, since the reactions of cracking involve principally dehydrogenation and cyclization reactions the antiknock properties of cracked motor fuel fractions are unusually good and the gasolines thus produced need only limited treatment to render them sufficiently stable for use as automotive engine fuel. Thus, very limited treatments remove the more reactive diolefins and, to some extent, the corrosive or malodorous sulfur compounds, or they may be sufficiently stabilized by the use of selective inhibitors. However, as the antiknock value of cracked gasolines is raised by more and more intensive cracking, the yields necessarily decrease on account of the loss of hydrogen, and a point is reached where the increase in antiknock value is more than counterbalanced by the decrease in yield so that further cracking is not economical.

In all cracking processes for the production of gasoline there is an incidental concurrent production of fixed gases which contain high percentages of olefinic constituents as well as paraffins and free hydrogen. For purposes of reference the following table shows the hydrocarbon compounds which have been definitely identified in cracked gas mixtures:

|    |            |             |
|----|------------|-------------|
| 50 | Methane,   | Butanes,    |
|    | Ethane,    | Butylenes,  |
|    | Ethylene,  | Pentanes,   |
|    | Acetylene, | Amylenes,   |
|    | Propane,   | Butadienes. |
| 55 | Propylene, |             |

The ratio of unsaturated hydrocarbons to paraffins depends, to a considerable extent, upon the conditions of cracking, the relatively high temperature and low pressure processes currently

designated as "vapor phase" processes favoring the production of olefins, and particularly ethylene, as conditions of great severity are employed. Since the total production of gases in cracking operations may run from 5 to as high as 20 per cent by weight of the stock cracked, it is obviously important to make some utilization of these gases and, if possible, reconver them into gasoline. The primary point of attack is obviously to condense or polymerize the olefins and this has been attempted by various thermal and catalytic processes which are more or less commercial at the present time. It is with an improvement in the art of catalytically polymerizing the olefins in cracked gas mixtures that the present invention is especially concerned.

In one specific embodiment, the present invention comprises subjecting hydrocarbon gas mixtures containing isobutylene to the action of catalysts comprising essentially a mono-metallic phosphate, particularly ortho-phosphates, which are selective in polymerizing the isobutylene to form 2,2,4-trimethyl pentene and perhaps, to some extent, isomers thereof by mixed polymerization, which is hydrogenatable to form the corresponding octane.

Experiments on olefin-containing gas mixtures, on olefin mixtures, and on individual olefins, have indicated that, of the normally gaseous olefins, isobutylene is most susceptible to polymerizing influences and that ethylene is the least susceptible. In catalytic processes, therefore, there is a tendency for the isobutylene to be removed under relatively mild conditions of temperature, pressure and catalytic influence, though there is usually some concurrent mixed polymerization in which the iso and normal butenes combine to form octenes. This reaction may occur, to some extent, in the present invention. Since the various isomers thus produced boil within rather close ranges of temperature, there may be considerable difficulty in separating them when only the dimer of isobutylene is desired in the product. The phenomenon of mixed polymerization, which produces compounds which may be considered to contaminate this pure dimer, is observed with various catalysts and particularly with phosphoric acid catalysts, either liquid or the so-called "solid" variety, which consists of a relatively inert siliceous carrier impregnated with an acid of phosphorus, usually the pyro acid or one closely approaching this in composition in most instances. By the use of the present process, however, in which mono-metallic ortho-phosphates are employed as catalysts, it has been found possible and practical to select conditions of temperature and pressure for many gas mixtures containing isobutylene under which sub-

stantially only the isobutylene is affected and the desired dimer, which may be readily hydrogenated to produce 2,2,4-trimethyl pentane, is produced in a state of comparative purity.

5 The preferred catalysts comprise the mono metallic-ortho phosphates of the alkali and the alkaline earth metals, though some of the so-called heavy metal compounds may be successfully employed. These compounds have a generally weaker polymerizing action than catalysts which comprise some acid phosphorus as their active constituent, on account of the partial replacement of the acid hydrogen by bases. Below are listed a few of the compounds which may be employed:

Ca(H<sub>2</sub>PO<sub>4</sub>)<sub>2</sub>.H<sub>2</sub>O..... Mono-calcium phosphate.  
Mg(H<sub>2</sub>PO<sub>4</sub>)<sub>2</sub>..... Mono-magnesium phosphate.  
Ba(H<sub>2</sub>PO<sub>4</sub>)<sub>2</sub>..... Mono-barium phosphate.  
20 Sr(H<sub>2</sub>PO<sub>4</sub>)<sub>2</sub>..... Mono-strontium phosphate.  
NaH<sub>2</sub>PO<sub>4</sub>.H<sub>2</sub>O..... Mono-sodium phosphate.  
KH<sub>2</sub>PO<sub>4</sub>..... Mono-potassium phosphate.

The mono alkali metal phosphates are soluble in water and normally best utilized after being mixed 25 with or deposited upon carriers from solution. Carriers which may be used are kieselguhr, crushed silica, and various types of silicates, particularly bentonite and montmorillonite clays, which may be molded or formed to produce pellets or special shapes. The alkaline earth phosphates are generally insoluble in water and are readily utilized in granular form in particle sizes within some definite mesh range, usually form 4 to 20.

35 In polymerizing isobutylene by the use of the preferred catalysts, they are most conveniently employed as filler in vertical cylindrical treating towers, the gas mixture to be treated being pre-heated to a suitable temperature and passed 40 downwardly through the bed of catalyst at an optimum rate for the selective removal of the isobutylene as the liquid dimer. The temperatures employed will vary within the approximate range of 250 to 550° F., depending upon the particular 45 catalyst used and the percentage of the isobutylene in the gas mixture. In the case of the calcium compound, which is easily procurable and quite effective, temperatures from 300 to 500° F. may be employed. The process is particularly 50 suitable for the treatment of the overhead products from stabilizers operating upon primary cracked distillates, which comprise principally hydrocarbons of three and four carbon atoms, including propane, propylene, butanes and butylenes, and in which isobutylene may occur from 55 approximately 5 to 15% concentration depending upon the character of the cracked distillate undergoing stabilization although gases direct from a cracking process may be treated. These mixtures may be pumped as liquids and vaporized 60 during passage through heating elements in which they are raised to the temperature found most suitable for the selective removal of isobutylene, using a catalyst selected from the present group. 65 The liquid dimer is readily separated from the unaffected residual gases and the latter may then be subjected to more severe conditions of temperature, pressure and catalytic influence, such as the solid phosphoric acid catalysts mentioned or to other polymerizing agent (and this is contemplated 70 within the scope of the process) in order

to produce further quantities of liquid polymers which may have a sufficiently high octane number to render them well suited to blending with gasolines inferior in antiknock value.

The dimer of isobutylene is readily hydrogenated under moderate conditions, such as a temperature of about 500° F. and a hydrogen pressure of 1000 lbs. per square inch, while using such catalysts as nickel oxide or the sulfides of the commoner elements in the sixth group of the periodic table, including chromium, molybdenum or tungsten. This step of the process may follow continuously from the other.

The following example is introduced to show the character of the results obtainable by the use 15 of the present process, although it is not intended to limit the scope of the invention in exact correspondence with the date presented.

A mixture of hydrocarbons constituting the overhead from a cracked gasoline stabilizer and 20 comprising 8% by volume (on a gas basis) of isobutylene was passed downwardly through a bed of granular mono-calcium-ortho-phosphate at a temperature of 350° F. and a pressure of 500 lbs. per square inch. Under these conditions the 25 dimer of isobutylene was produced in a condition of 95% purity, the additional 5% being a mixture of dimers which were removable by a fairly careful fractionation, the normal butylenes and propylene being substantially unaffected by the 30 treatment. Good results were also produced when cracked gases direct were treated with the phosphate catalyst and combination treatment e. g. following the present process by the use of a stronger polymerizing agent to polymerize the 35 residual olefins also gave good results.

The character of the present invention and the definitely practical value thereof will be evident from the foregoing specification and single instance of results obtained, though neither section is intended to be unduly limiting.

I claim as my invention:

1. A process for producing iso-octene from a hydrocarbon gas mixture containing isobutylene and other polymerizable gaseous olefins, which 45 comprises subjecting the mixture at a temperature of from 250 to 550° F. to the action of a mono-metallic-ortho-phosphate to selectively polymerize isobutylene from the mixture and separating the resultant polymer from the unpolymerized gases.

2. A process for producing iso-octene from a hydrocarbon gas mixture containing isobutylene and other polymerizable gaseous olefins, which 55 comprises subjecting the mixture at a temperature of from 250 to 550° F. to the action of a mono-metallic-ortho-phosphate of an alkaline metal to selectively polymerize isobutylene from the mixture, and separating the resultant polymer from the unpolymerized gases.

3. A process for producing iso-octene from a hydrocarbon gas mixture containing isobutylene and other polymerizable gaseous olefins, which 65 comprises subjecting the mixture at a temperature of from 250 to 550° F. to the action of a mono-calcium-ortho-phosphate to selectively polymerize isobutylene from the mixture, and separating the resultant polymer from the unpolymerized gases.